# EUROPEAN PATENT APPLICATION

(11) **EP 3 441 988 A1**
(43) Date of publication of application: **13.02.2019**
(21) Application number: 18187975.0
(22) Date of filing: 08.08.2018
(51) Int. Cl.: H01F 1/057

(54) **A SINTERED R-T-B BASED PERMANENT MAGNET**

(30) Priority: 10.08.2017 CN 201710678374
(71) Applicant: Yantai Shougang Magnetic Materials Inc., 265500 Yantai (CN)
(72) Inventor: DING, Kaihong, Yantai, 265500 (CN); PENG, Zhongjie, Yantai, 265500 (CN); DONG, Zhanji, Yantai, 265500 (CN); CHEN, Xiulei, Yantai, 265500 (CN)
(74) Representative: Gulde & Partner

(57) **Abstract**

The present invention provides a sintered R-T-B based permanent magnet characterized by:
- a crystal structure with a first-type grain boundary in the direction of the easy-orientation axis of the magnet and a second-type grain boundary perpendicular to the easy-orientation axis of the magnet, both being a face-centered cubic structure (fcc); and
- a first triple junction area phase including an Al and Ga element rich rare-earth phase with an amorphous crystal structure, whose composition satisfies the condition (atomic percentage): 65%≤Pr+Nd≤88%, 10%≤Al+Ga≤25%, O≤10%, and other elements, Fe+Cu+Co≤2%; and/or
a second triple junction area phase including a Cu and Ga rich rare-earth phase with a densely packed hexagonal crystal structure (dhcp), whose composition satisfies the condition (atomic percentage): 50%≤Pr+Nd≤70%, 10%≤Cu+Ga≤20%, 10%≤Fe+Co≤20%, and O≤10%.

## Description

### BACKGROUND OF THE INVENTION

### 1. Field of the invention

The present invention relates to an R-T-B based sintered permanent magnet having a novel microstructure.

### 2. Description of the prior art

Nowadays, R-T-B based sintered permanent magnet materials are used in wind power generation, air conditioning, elevators, and new energy vehicles more and more widely. However, due to the high price of heavy rare earth elements Dy and Tb, the demand for production of the permanent magnet with high coercivity but with less or no addition of heavy rare earth element is getting higher and higher.

In order to save the use of heavy rare earth and maximize the coercivity increment of the magnets, grain boundary diffusion techniques of pure metals, heavy rare earth elements, two-phase or multiphase alloys, oxide or fluoride can be used. The advantage of this technology is that by adding only less than 1% of the heavy rare earth of the magnet, the coercivity increment will as same as a conventional process magnet contained 5% to 10% heavy rare earth elements, so the effect of saving the heavy rare earth is significant. However, the biggest disadvantage of grain boundary diffusion process is that it cannot be applied to products with a thickness greater than 5mm because the diffusion process is greatly affected by the thickness of the product. Therefore, in some areas, such as HEV, the application of this product is limited.

It is reported by the patent (Japanese Patent 2015-5767788) that by addition of 0.5% Ga to a sintered NdFeB magnet without heavy rare earth added can significantly increase the coercivity because Nd6(FeGa)14 phase (named 6:14 phase) is formed in the triple junction areas. Also, it is reported by the paper (T.T. Sasaki et al. Scripta Materialia 113 (2016) 218-221) that, the grain boundary width is increased by the formation of the 6:14 phase. This kind of thick grain boundary phase makes a strong exchange decoupling between neighbouring grains and attribute to a higher coercivity.

Although the coercivity is increased by the formation of 6:14 phase, too much rare earth elements are introduced into the 6:14 phase, Pr, and Nd, for example. Further, by making the grain boundary thickness and rare earth elements distribution uniform, the squareness of the magnet becomes worse. In addition, although the price of the Ga element is lower than that of the heavy rare earth element, Tb, and Dy, for example, it is much higher than the price of the Nd and Pr element. Therefore, it is necessary to add as little Ga as possible to the magnet while still keeping high coercivity.

### SUMMARY OF THE INVENTION

The present invention shall overcome the deficiencies of the prior process mentioned above and provide a sintered heavy rare earth free NdFeB magnet with high coercivity.

According to the present invention, there is provided a sintered R-T-B based permanent magnet characterized by:
- a crystal structure with a first-type grain boundary in the direction of the easy-orientation axis of the magnet and a second-type grain boundary perpendicular to the easy-orientation axis of the magnet, both being a face-centered cubic structure (fcc);
- a first triple junction area phase including an Al and Ga element rich rare-earth phase with an amorphous crystal structure, whose composition satisfies the condition (atomic percentage): 65%≤Pr+Nd≤88%, 10%≤Al+Ga≤25%, O≤10%, and other elements, Fe+Cu+Co≤2%; and/or
   a second triple junction area phase including a Cu and Ga rich rare-earth phase with a densely packed hexagonal crystal structure (dhcp), whose composition satisfies the condition (atomic percentage): 50%≤Pr+Nd≤70%, 10%≤Cu+Ga≤20%, 10%≤Fe+Co≤20%, and O≤10%.

Thus, the magnet shows a specific microstructure. Specifically, the reasonable selection of the alloy composition ensures the formation of a matrix phase which enforces the remanence. Besides, the formation of a grain boundary phase is ensured which prevents demagnetization of the magnet.

Furthermore, Cu element is added to the alloy to form a R-Cu (R means rear earth elements) phase. During the annealing process, the melting temperature will decrease by the presence of the R-Cu phase. Then the R-Cu phase will infiltrate into the grain boundaries to form R-rich layers to enhance the coercivity.

Furthermore, Cu element is added to the alloy to increase the Curie temperature and the temperature dependency of the coercivity.

Furthermore, Al and Ga element is added to the alloy to improve the wettability of the grain boundary phase, making the Pr and Nd element infiltrate to the grain boundary easily and enhance the coercivity.

Furthermore, the coercivity and squareness of the magnets according to the present invention are higher than 20kOe and higher than 0.96, respectively.

In general, the present invention provides a sintered R-T-B based magnet whose first-type grain boundary phase (in the direction of the easy-orientation axis) and second-type grain boundary phase (perpendicular to the easy-orientation axis) are both of a face-centered cubic structure (fcc).

The magnet further includes the first triple junction area phase: the relatively high content of Al-Ga element rich rare-earth phase, with an amorphous crystal structure, whose composition meet the relationship (atomic percentage): 65%≤Pr+Nd≤88%, 10%≤Al+Ga≤25%, O≤10%, and other elements, Fe+Cu+Co≤2%.

In alternative or in addition, the magnets further include the second triple junction area phase: relatively high Cu+Ga content, with a densely packed hexagonal crystal structure (dhcp), and the composition satisfies the relationship (atomic percentage): 50%≤Pr+Nd≤70%, 10%≤ Cu+Ga≤20%, 10%≤Fe+Co≤20%, and O≤10%.

### BRIEF DESCRIPTION OF THE FIGURES

Figure 1 is the demagnetization curve of example 1 at room temperature.
Figure 2 is the SEM image of example 1.
Figure 3 is the TEM image and electron diffraction spot of the grain boundary parallel to the easy orientation axis of example 1.
Figure 4 is the TEM image and electron diffraction spot of the grain boundary vertical to the easy orientation axis of example 1.
Figure 5 is the EDS mapping of the triple junction area of example 1.
Figure 6 is the TEM electron diffraction spot of example 1, (a) is an amorphous structure and (b) is a dhcp structure.
Figure 7 is the TEM image and electron diffraction spot of the grain boundary parallel to the easy orientation axis of example 2.
Figure 8 is the TEM image and electron diffraction spot of the grain boundary vertical to the easy orientation axis of example 2.
Figure 9 is the EDS mapping of the triple junction area of example 2.
Figure 10 is the TEM electron diffraction spot of example 2, (c) is an amorphous structure and (d) is a dhcp structure.
Figure 11 is the the TEM image and electron diffraction spot of the grain boundary parallel to the easy orientation axis of example 3.
Figure 12 is the TEM image and electron diffraction spot of the grain boundary vertical to the easy orientation axis of example 3.
Figure 13 is the EDS mapping of the triple junction area of example 3.
Figure 14 is the TEM electron diffraction spot of example 3, (e) is an amorphous structure and (f) is a dhcp structure.

### DETAILED DESCRIPTION OF THE INVENTION

In the following, a detailed description for the preparation of a heavy rear earth element free sintered NdFeB based magnet is provided.

The atomic percent nominal composition of the alloy is 14.2%∼15.6% of Pr and Nd, 4.9%∼7.3% of B, 0.9%∼2.0% of Al, 0.7%∼1.3% of Co, 0.2%∼0.5% of Cu, 0.1%∼0.4% of Ga, and the balance amount of Fe. The weight percent nominal composition of the alloy is 31%∼34% of Pr and Nd, 0.8%∼1.2% of B, 0.4%∼0.8% of Al, 0.6%∼1.2% of Co, 0.2%∼0.5% of Cu, 0.1%∼0.4% of Ga, and the balance amount of Fe.

In generell, the alloy was made into flakes with the thickness of 0.2∼0.5mm using a scripting casting process.

The flakes were transferred into a hydrogen desorption furnace and broken into coarse powders. The hydrogen absorbing time was 3.5 hours under a 0.15∼0.3Mpa hydrogen pressure and the hydrogen decrepitation temperature was 550°C.

After the decrepitation process, 0.05∼0.5 wt.% of usual lubricant was added into the coarse powders. Then the coarse powders were pulverized in a jet milling machine to prepare a fine powder which average grain size (D50) was 2.0∼3.5µm.

Another amount of 0.03∼0.2wt.% usual lubricant was added into the fine powder after pulverizing and then mixed in a blender mixer for 1∼2 hours. After that, the fine powder was compressed into green compacts with a magnetic field of 2.0∼2.5T under an Ar gas atmosphere.

After the model compressing process, the green compacts were put into a high vacuum furnace and sintering for 6-15 hours under 880∼1030°C to get bulk magnets. After cooling down to room temperature, the bulk magnets were annealed at 780∼860°C for 3 hours for the first step and were annealed at 480∼550°C for 2∼8 hours for the second step. During the sintering and annealing process, the value of the furnace vacuum was below 5×10⁻²Pₐ.

During all the processing steps, the oxygen and nitrogen contents were controlled strictly to ensure that the C, O and N contents in the final bulk magnet meet C≤800ppm, O≤800ppm, and N≤200ppm.

### EXAMPLES

Example 1: An alloy with an atomic percent of (Pr+Nd)15-B5.6-Co1.1-Cu0.4-Al1.0-Ga0.2-Fe bal., respectively with a weight percent of (Pr+Nd)32.5-B0.9-Co1.0-Cu0.4-Al0.4-Ga0.2-Fe bal. was prepared. A Scrip casting method was used for getting flakes with a thickness of 0.2∼0.5mm. The flakes were subjected into a hydrogen desorption furnace and were broken into coarse powders. The hydrogen absorbing time was 3.5 hours under a 0.2Mpa hydrogen pressure and the hydrogen decrepitation temperature was 550°C; After the decrepitation process, 0.1 wt.% of usual lubricant was added into the coarse powders, then the coarse powders were pulverized in a jet milling machine to prepare the fine powder which average grain size (D50) was 2.8µm. Another amount of 0.05wt.% of the usual lubricant was added into the fine powder after pulverizing and then mixed in a blender mixer for 2 hours. After that, the fine powder was compressed into green compacts with a magnetic field of 2.0T under an Ar gas atmosphere. After the model compressing process, the green compacts were put into a high vacuum furnace and were sintered for 6 hours under 920°C to get bulk magnets. After cooling down to room temperature, the bulk magnets were annealed at 850°C for 3 hours in a first first step and were annealed at 525°C for 2 hours in a second step. The content of C, O, and N of the final bulk magnet were 750ppm, 600ppm, and 150ppm, respectively.

In order to compare the implementation effect, the bulk magnets of Examples 2 and 3 were prepared by the same process described above for Example 1.

Transmission electron microscopy (TEM) was used for analyzing the microstructure of the examples. As is shown in Table 1 and the (scanning electron microscope) SEM images and SAED (selected area electron diffraction) patterns, it is confirmed that all the AB plane and C plane faces can be indexed as an fcc structure. At the same time, TEM equipped with an energy dispersive spectroscopy (EDS) detector was used for analyzing the microstructure and composition of the triple junction areas of each example. It has been found that two kinds of areas with different composition and crystalline structure exist. Detailed data are summarized in Table 2 and the TEM images are described as follows.

**Table 1 - Magnet composition and crystalline structure of each example**

| Examples | | Pr | Nd | B | Co | Cu | Al | Ga | Fe | AB plane | C plane |
|---|---|---|---|---|---|---|---|---|---|---|---|
| 1 | wt.% | 7.0 | 25.5 | 0.9 | 1.0 | 0.4 | 0.4 | 0.2 | Balance | fcc Structure | fcc Structure |
| | at.% | 3.3 | 11.7 | 5.6 | 1.1 | 0.4 | 1.0 | 0.2 | | | |
| 2 | wt.% | 6.6 | 24.3 | 0.8 | 0.7 | 0.2 | 0.4 | 0.1 | | | |
| | at.% | 3.1 | 11.1 | 5.0 | 0.8 | 0.2 | 0.9 | 0.1 | | | |
| 3 | wt.% | 7.3 | 26.7 | 1.2 | 1.2 | 0.5 | 0.7 | 0.4 | | | |
| | at.% | 3.4 | 12.2 | 7.3 | 1.3 | 0.5 | 1.8 | 0.4 | | | |

**Table 2 - Composition of the triple junction area of each example**

| Areas | Examples | | Pr+Nd | Co | Cu | A1 | Ga | Fe | 0 |
|---|---|---|---|---|---|---|---|---|---|
| dhcp phase | 1 | wt.% | 82.1 | 1.5 | 5.1 | 0.6 | 3.3 | 6.6 | 0.8 |
| | | at.% | 62.4 | 2.7 | 8.8 | 2.6 | 5.1 | 13.0 | 5.4 |
| | 2 | wt.% | 79.5 | 1.5 | 3.8 | 1.4 | 3.4 | 9.1 | 1.4 |
| | | at.% | 56.0 | 2.5 | 6.1 | 5.2 | 4.9 | 16.5 | 8.8 |
| | 3 | wt.% | 84.2 | 1.3 | 5.5 | 0.6 | 4.3 | 3.8 | 0.2 |
| | | at.% | 68.0 | 2.6 | 10.1 | 2.7 | 7.2 | 7.9 | 1.5 |
| amorphous phase | 1 | wt.% | 89.9 | 0.2 | 0.4 | 1.6 | 6.6 | 0.7 | 0.7 |
| | | at.% | 74.1 | 0.3 | 0.8 | 7.1 | 11.2 | 1.4 | 5.1 |
| | 2 | wt.% | 85.2 | 0.1 | 0.4 | 1.5 | 11.2 | 0.6 | 1.1 |
| | | at.% | 66.2 | 0.1 | 0.7 | 6. 2 | 17.8 | 1.1 | 7.9 |
| | 3 | wt.% | 93.7 | 0.1 | 0.1 | 0.9 | 5.0 | 0.1 | 0.1 |
| | | at.% | 85.1 | 0.2 | 0.2 | 4.5 | 9.3 | 0.3 | 0.4 |

Fig.1 is the magnet B-H curve of Example 1. Dashed line and solid line are the B-H curves of as sintered and after annealed magnet respectively. The Br and the Hcj of the as-sintered magnet are 13.05kGs and 14.8kOe respectively, and the Br, Hcj, and squareness of the after annealed magnet are 13.0kGs, 20.1kOe, and 0.96 respectively, at room temperature.

Fig.2 is the SEM image of Example 1. It can be seen that the average grain size of the compact magnet after sintering is roughly 3.5µm. Depending on the contrast, the matrix phase with dark contrast is a Nd₂Fe₁₄B phase, the white, the thin and long area is grain boundary Nd-rich phase, and the residual white area is triple junction Nd-rich phase. Furthermore, when zooming in the triple junction Nd-rich phase, there are still some different areas with different contrast. That means, some phases with different structure should exist in the triple junction areas.

According to the recent literature, the composition and structure of the grain boundary phase of the sintered NdFeB magnet will be different due to the angle between the grain boundary and the easy-orientation axis. Typically, according to the different values of the angle, it can be divided into two kinds, one is named AB plane, which is paralyzed to the easy orientation axis, the other one is named C plane, which is vertical to the easy orientation. Fig. 3 and Fig. 4 show the transmission electron micrographs and electron diffraction spots of two typical grain boundary phases according to the above principle. The former is AB plane and the latter is C plane. According to analysis of the transmission electron microscopy electron diffraction spot of the corresponding grain boundary phase, and according to the calculation results of the lattice constant, it is clear that the grain boundary phases of the AB plane and the C plane in the magnet are all fcc structures (measured value lattice constant of a is about 0.56 nm). The thickness of the grain boundary phase is about 3 nanometers.

Similarly, in this example, a TEM is used to obtain detailed composition and structure of the triple junction areas at high magnification. Fig. 5 is an EDS mapping photograph showing the element distribution by the EDS component of the transmission electron microscope. It is obviously in Fig. 5 that the triple junction area includes a region in which the Al element and the Ga element content are particularly high, that is, marked region (a) in the figure. Fig. 6 is an electron diffraction spot corresponding to the regions (a) and (b), respectively, and it can be seen that the region (a) is an amorphous phase structure, and the region (b) is a close-packed hexagonal crystal structure (dhcp).

Fig.7 and Fig. 8 are the high-resolution transmission electron micrographs and corresponding electron diffraction spots taken from the grain boundary along the easy orientation axis and the grain boundary vertical to the easy orientation axis of Example 2, respectively. According to the calculation of the lattice constant, the grain boundaries are all fcc structures. Fig. 9 and Fig. 10 are the EDS mapping result and the electron diffraction spot photograph taken from the triple junction area of Example 2 at high magnification, respectively. It is found that the region (c) is an amorphous structure rich in Al and Ga, and the region (d) is a close-packed hexagonal structure rich in Cu and Ga.

Correspondingly, Fig. 11 and Fig. 12 are the high-resolution transmission electron micrographs and corresponding electron diffraction spots of the grain boundary along the easy orientation axis and vertical to the easy orientation axis of Example 3, respectively. Similar to the calculation results of Example 1 and Example 2, both grain boundaries are fcc structures. Fig. 13 and Fig. 14 are the EDS mapping result and the electron diffraction spot photograph taken from the triple junction area of Example 3 at high magnification, respectively. It is found that the region (e) is an amorphous structure rich in Al and Ga, and the region (f) is a close-packed hexagonal structure rich in Cu and Ga.

In addition, in this example, it can be clearly seen that the thickness of the grain boundary of the annealed magnet is uniform and continuous, that maybe the reason of the better squareness in this example compared with the magnet of high Ga. In addition, the dhcp structure can be found in the examples, which is also one of the differences between the high Ga magnet and the examples in the present patent. As the oxygen content increases, the structure of the Nd-rich phase will change gradually: in the case of low oxygen, it is the dhcp phase, with the oxygen content increase, the structure will change to fcc phase, and finally change to the hcp phase. Different with NdOₓ phase and cubic phase structure of Nd₂O₃ phase, the Nd-rich phase with the close-packed hexagonal crystal structure (dhcp) is much easier to react with Cu to form Nd-Cu rich phase, because of the low oxygen content. And after the annealing process, the element flows toward the grain boundary phase to form a sufficient grain boundary phase, thereby increasing the coercivity of the magnet. Therefore, in order to obtain this special microstructure, strict control of the content of C, O, and N in the magnet is also one of the necessary means to make NdFeB sintered magnet with high coercivity.

## Claims

1. A sintered R-T-B based permanent magnet **characterized by**:
- a crystal structure with a first-type grain boundary in the direction of the easy-orientation axis of the magnet and a second-type grain boundary perpendicular to the easy-orientation axis of the magnet, both being a face-centered cubic structure (fcc); and
- a first triple junction area phase including an Al and Ga element rich rare-earth phase with an amorphous crystal structure, whose composition satisfies the condition (atomic percentage): 65%≤Pr+Nd≤88%, 10%≤Al+Ga≤25%, O≤10%, and other elements, Fe+Cu+Co≤2%; and/or
a second triple junction area phase including a Cu and Ga rich rare-earth phase with a densely packed hexagonal crystal structure (dhcp), whose composition satisfies the condition (atomic percentage): 50%≤Pr+Nd≤70%, 10%≤Cu+Ga≤20%, 10%≤Fe+Co≤20%, and O≤10%.
